

May 14, 1929.

E. GATHMANN

1,712,608

INGOT

Original Filed March 15, 1927



Fig. 2.



Fig. 3.



Fig. 4.



Fig. 6.

Inventor  
Emil Gathmann  
by his Attorneys  
Baldwin Wright

## UNITED STATES PATENT OFFICE.

EMIL GATHMANN, OF BALTIMORE, MARYLAND.

## INGOT.

Original application filed March 15, 1927, Serial No. 175,527. Divided and this application filed January 20, 1928. Serial No. 248,176.

The application for this patent is a division of my application for patent filed March 15, 1927, Serial No. 175,527, patented February 28, 1928, No. 1,661,039.

5 This invention relates to the manufacture of ingots, the metal of which contracts during solidification from the molten to the solid, the horizontal length and width of which ingots are materially greater than the vertical height. Such ingots are more economically reduced by forging and rolling mill operations to plates, sheets and various other units than are ingots made by the more widely used method of so-called vertical casting.

10 15 Prior to my invention ingots have been cast in what are known to those familiar with the art as horizontal molds, i. e., molds in which the longitudinal axis of the mold chamber is disposed horizontally. In the use of such molds, however, longitudinally extending pipes or shrinkage cavities have been formed in the ingot, and in steel and other alloyed metals cast in such molds segregation of the various elements has occurred to a dangerous

20 25 degree, so that when the ingot is rolled into commercial shapes or units, some parts are sound and uniform while others are unsound or have widely varying physical and chemical characteristics, thus causing stresses to be set up in the semi-finished product, which render it liable to break or split during the process of manufacture or in its use.

By my improvements I am enabled to produce an ingot of the horizontally cast type, 35 which is free from pipe and shrinkage cracks and in which the segregation may be to a great extent controlled. For certain products it is desirable to reduce segregation to a minimum, which I have made possible by 40 reducing the depth of the ingot relative to its width to induce rapid freezing of the entire mass. For certain other products, such as boiler plate, segregation can be distributed substantially evenly over the upper plane of 45 the ingot by providing any well-known means (such as coke dust, powdered graphite or the like spread upon the top of the molten metal while the ingot is being cast) for retaining the metal molten at its upper surface for the 50 desired length of time to obtain the amount of segregation required for the particular product.

The mold made in accordance with my invention preferably has a long, horizontally- 55 arranged major axis and a relatively nar-

rower transverse axis. The height or depth of the mold chamber is less than its width for reasons hereinafter explained. The side walls defining the ingot-forming chamber preferably gradually decrease in thickness 60 upwardly and the bottom wall, which is relatively thicker or more heat-absorptive than the side walls, is formed with a camber or rise which projects into the mold chamber in such a manner as to absorb heat more rapidly 65 from the middle or central longitudinal section of the molten metal than from adjacent portions thereof, thereby causing the metal of the ingot to solidify vertically in its middle and adjoining portions in a substantially uniform manner and more rapidly than it is being solidified laterally or horizontally 70 from the side walls of the mold. Experience has demonstrated that when the mold walls have these characteristics and the chamber 75 is properly dimensioned, the freezing or solidifying of the molten metal will be completed in less time for a given mass of metal than has heretofore been possible and the shrinkage of the mass will be of such a character that no pipe is formed either at the top or at the ends of the ingot and that segregation, due to the rapid rate of solidification of the molten metal, will be readily controlled.

My improvements are illustrated in the accompanying drawings, in which—

Figure 1 is a perspective view of a horizontal mold made in accordance with my invention, portions of the mold being omitted for convenience of illustration.

Figure 2 shows a vertical transverse section on lines 2—2 of Figure 1.

Figure 3 shows a section similar to that shown in Figure 2 with the solidified ingot shown in cross section in the mold cavity.

Figure 4 shows a longitudinal section of the mold on lines 4—4 of Figure 1 and illustrates also a longitudinal central section of the ingot cast in the mold.

Figure 5 is an enlarged view in perspective of a portion of the ingot.

Figure 6 is a perspective view of a portion of a plate or sheet rolled from an ingot such as shown in Figure 5.

The mold made in accordance with my invention is preferably of cast iron, which is commonly used in the manufacture of various types of ingot molds, the chamber walls being formed as smooth as the state of the art permits.

As is well-known to those skilled in the art, well deoxidized molten steel freezes and solidifies upwardly and inwardly from the mold chamber walls, usually through formation of dendritic crystals, until solidification is complete.

In vertical molds of now well-known design, this solidifying process of the ingot is so controlled by means of big end up mold 10 chambers and refractory shrink head casings that the so-called pipe or shrinkage cavity is greatly reduced and confined to a relatively small part of the ingot at its top. In the casting of ingots in horizontal molds, 15 however, a decided shrinkage pipe, cavity or crevice has heretofore been formed, which usually extends longitudinally from one end of the ingot to the other, being deepest and most pronounced near the center of the mass 20 of the ingot, which is always last to cool and solidify, at which zone segregation is likewise concentrated.

By my invention I so shape the mold chamber that the molten metal of the ingot 25 will solidify in its central longitudinal portion in substantially the same period of time as the side or surrounding portions and the ingot is so formed that what is known as cleavage cones and ingotism or the formation 30 of large crystals in the structure of the ingot are greatly reduced. The bottom or base of the ingot surface being inwardly bellied or cambered to an extent proportional to the width and depth of the mold chamber and 35 in ratio to the volume of the shrinkage of the metal forming the ingot during solidification, the formation of shrinkage cavities or pipes is prevented by compensating for and forcing the contraction of the metal in 40 vertical planes during solidification. A slightly dished or cambered portion at the upper face of the ingot is sometimes formed therein, but concentrated shrinkage cavities or piped zones are entirely prevented. In 45 this way a great saving is effected, as the percentage of sound metal which can be rolled or forged into commercial shapes is approximately the entire ingot, less only the usual scale and trimming loss of 4% to 6%.

50 An important feature of the invention is that the walls defining the mold chamber are of such contour and heat absorptive quality that the molten metal will cool, solidify and shrink in a substantially vertical direction 55 from the bottom upward in approximately the same period of time at all vertical planes, as the depth of the liquid ingot metal in the mold chamber at its central longitudinal portion is proportionately less and the cooling action of the mold walls greater than at 60 adjacent portions of the chamber.

The drawings illustrate one way of constructing a mold in accordance with my invention. The mold is made of cast iron of 65 the kind usually employed. The bottom B

of the mold is relatively thick and heavy and the side walls A, which are materially thinner and less heat absorptive, gradually decrease in thickness from their lower to their upper ends, thus insuring that the 70 solidification of the molten metal of the ingot will be progressively upwards, the same rule applying in the formation of the side walls of the horizontal molds as applies in the formation of side walls of vertical molds. 75 The bottom wall of my horizontal mold, however, differs from the bottom wall of other molds. It will be observed that the bottom wall, in addition to being relatively thick and heavy and thus more heat absor- 80 pitive than the side walls, is formed with a longitudinal rise or camber X, which projects to its highest part at the central or middle longitudinal portion of the mold chamber, so that as the molten metal cools, shrinks 85 and solidifies coincidently in the middle portion of the mold with that of all adjoining portions, the entire mass of metal becomes solidified without pipe or shrinkage cavity being formed therein. The rise X may have 90 various contours but is preferably cambered in the form of a convex arc as shown, the amount of this rise being governed by the depth and width of mold chamber and the character of the ingot metal for which the 95 mold is designed.

As previously stated, the height of the mold chamber or that part thereof in which the casting is made, is less than its width. I have found that the width should considerably exceed the depth of the chamber in order to obtain the best results. The exact ratio depends upon the type of material being cast and the product for which the ingot is intended, e. g., for low-carbon de-gassified 100 steel, which solidifies relatively rapidly, a mold of the following dimensions might be used for sheet bar product.

If the width of the mold chamber at its 110 top is 12", the greatest height of the chamber should be approximately 8", while its height from the top of the rise X should be about 7". The over-all height of the mold should be approximately 13", the distance from the bottom face of the mold to the top of the rise 115 X thus being about 6". The taper of the mold chamber from top to bottom should be approximately  $\frac{1}{2}$ ".

These relative dimensions have given satisfactory results in actual test, but may and 120 should be varied to correspond with specific conditions and requirements. The mold may be of any desired length within limitation. Any length to which the metal can flow without danger of laps or cold shuts may be 125 utilized.

It will be understood by those familiar with the art that the liquid metal of an ingot solidifying in a metallic mold is invariably hottest 130 for a longer period of time at the central or

middle portion of its mass than at adjacent portions of the ingot unless means are utilized to accelerate its cooling. By my improvement there is less vertical height of ingot to cool at the center of the mass than at adjacent transverse parts, so that the rate of vertical cooling, within the limits specified, can be adjusted to obtain uniform solidification.

The method of teeming or pouring the metal into my improved type of mold and the stripping of the ingot therefrom is not a part of this invention. Various well-known methods have been found satisfactory.

Referring to Figure 5 of the drawings, I have illustrated by dotted lines, *a*, *b*, *c*, and *d*, the manner in which solidification of the ingot occurs.

In Figure 6 of the drawings I have shown in perspective a portion of a plate showing the uniformly segregated zone portion in dotted lines, this portion having been the last of the ingot to solidify.

It will be observed that the ingot formed in the manner hereinbefore described, has two primary side walls, that is, the bottom and top of the ingot, and four secondary walls, namely, the longitudinal sides and the ends. It will also be observed, by reference to Figure 5 particularly, that all corners are well rounded. By such a construction most efficient heating and rolling can be obtained without danger of burning or cracking during these operations.

I claim as my invention:

1. An ingot of slab-like contour, the depth of which slab is less than its width or length, one of the primary sides of larger area being concaved to a depth of not over one-fourth but to at least one-eighth of the thickness of said ingot.

2. A horizontally-cast ingot, the length of which is greater than its width and the depth of which is less than its width, one of the sides of a larger area being concaved to a depth between one-eighth and one-fourth of the thickness of the ingot.

3. An ingot of slab-like contour formed of a metal that contracts in volume during solidification, said ingot having a length that is greater than its width and a depth which is less than its width, one of the sides of larger area of said ingot being concaved to a depth of at least one-eighth but not exceeding one-fourth of the thickness of said ingot.

4. A horizontally-cast ingot formed of a metal that contracts in volume during solidification, the length of which is greater than its width and the depth of which is less than its width, one of the sides of larger area being

concaved to an extent not exceeding one-fourth of the depth of the ingot and the ingot throughout its entire structure being free from pipe.

5. A horizontally-cast ingot formed of a metal that contracts in volume during solidification, the length of said ingot being greater than its width and the width of the ingot being greater than its depth and the bottom surface of the ingot being formed of a concave or inwardly-cambered contour, the depth of said concavity being more than one-eighth, but less than one-fourth of the thickness of the ingot.

6. A horizontally-cast ingot formed of a metal that contracts in volume during solidification, the length of said ingot being greater than its width and the width of which ingot is materially greater than its thickness and the two major or primary surfaces of which is formed of a concave or inwardly-cambered contour, the thickness of said ingot being less at its central longitudinal section than at adjacent longitudinal portions.

7. A horizontally cast ingot, the length of which is greater than its width and the depth of which is less than its width, both of the sides of larger area being concave, the width of said ingot being at least four times its depth.

8. A long thin slag ingot having a shallow concaved lower portion and a slightly concaved upper portion, the opposite side portions of the ingot being inclined outwardly from bottom to top.

9. A long thin slab ingot having a shallow concaved lower portion and a slightly concaved upper portion the opposite side portions of the ingot being inclined outwardly from bottom to top, and the four corners of said ingot being rounded.

10. A metallic ingot of slab-like contour, the bottom of which is concaved in a curve of substantially uniform radius, the top of which ingot is slightly concaved and the sides of which are inclined outwardly from bottom to top.

11. A metallic ingot of slab-like contour and having oppositely disposed side walls connected by an inwardly dished bottom wall and rounded corner walls interposed between the bottom walls and the lower edges of the respective side walls, said dished bottom wall having a substantially uniform curvature from one of said corner walls to the other of said corner walls.

In testimony whereof, I have hereunto subscribed my name.

EMIL GATHMANN.